

Sept. 28, 1954

W. C. LILLIENDAHL ET AL

2,690,421

## ELECTROLYTIC PRODUCTION OF URANIUM POWDER

Filed March 6, 1943

2 Sheets-Sheet 1



Sept. 28, 1954

W. C. LILLIENDAHL ET AL

2,690,421

ELECTROLYTIC PRODUCTION OF URANIUM POWDER

Filed March 6, 1943

2 Sheets-Sheet 2



## UNITED STATES PATENT OFFICE

2,690,421

## ELECTROLYTIC PRODUCTION OF URANIUM POWDER

William C. Lilliendahl, Mountain Lakes, Donald Wroughton, East Orange, Rudolph Nagy, Bloomfield, and John W. Marden, East Orange, N. J., assignors to the United States of America as represented by the United States Atomic Energy Commission

Application March 6, 1943, Serial No. 478,270

3 Claims. (Cl. 204—10)

1

This invention relates to the manufacture of uranium, and more particularly to the commercial production of said material in powdered form.

The principal object of our invention, generally considered, is to produce uranium of exceedingly high purity on a commercial scale.

Another object of our invention is the large scale production of an oxygen-free halide salt of uranium containing no undesirable impurities.

A further object of our invention is the electrolysis of a bath composed of a pure halide of uranium fused in a mixture of chlorides held at such a temperature that the metal uranium is deposited as a coarse powder on a cathode of refractory material such as molybdenum.

A still further object of our invention is the removal of the uranium-containing deposits from the cathode and treatment thereof to conserve the uranium powder produced.

Other objects and advantages of the invention, relating to the particular arrangement and construction of the various parts, will become apparent as the description proceeds.

In the drawing illustrating our invention:

Fig. 1 is a flow diagram showing how potassium uranous fluoride is formed on a commercial scale and then washed, dried, and electrolyzed to produce uranium powder embedded in other electrolyte material; and how said electrolyzed material is removed from the cathode, crushed, ground, washed in a tumbling barrel, ground, again treated in a tumbling barrel, filtered, and dried in vacuum, after which the metal powder may be pressed, and sintered and/or fused to produce the finished product.

Fig. 2 is a vertical sectional view illustrating apparatus for introducing "green salt" or other uranium compound to be electrolyzed, into the molten bath below the surface thereof.

Fig. 3 is a view corresponding to Fig. 2 but showing an alternative apparatus for introducing pressed blocks of "green salt" beneath the surface of the bath.

Fig. 4 is a view corresponding to Fig. 3 but showing a further alternative apparatus, whereby "green salt" may be introduced as a steady stream beneath the surface.

Fig. 5 illustrates another embodiment for introducing "green salt" into the bath, while protecting the former from decomposition.

Fig. 6 is a plan of alternative apparatus for electrolyzing the "green salt" or other uranium compound.

Fig. 7 is a vertical sectional view of an elec-

2

trode, alternative to that shown in Fig. 1, in a fused bath held in its associated crucible.

Fig. 8 is a view corresponding to Fig. 7, but showing an ordinary type of central electrode functioning as a cathode, with a modified form of crucible associated therewith.

Fig. 9 is a view corresponding to Fig. 8 but showing another modification for the same purpose.

10 Fig. 10 is a transverse sectional view on the line X—X of Fig. 9, in the direction of the arrows; and

Fig. 11 is a vertical sectional view of a water cooled container for smothering coated cathodes in salt.

*Making "green salt"*

In accordance with our invention we first prepare potassium uranous fluoride,  $KUF_5$  (called "green salt," and in which uranium is tetravalent) by a photochemical reduction, preferably using sunlight, of a solution containing a uranium salt such as the nitrate (in which the uranium has a valency of six), potassium fluoride, hydrofluoric acid, and a reducing agent such as formic acid or sucrose. The potassium uranous fluoride is precipitated as a heavy green salt and collects at the bottom of the vessel from which the liquor may be decanted and the desired product removed, filtered, washed, and dried to yield a salt suitable for the electrolysis operation.

The reducing agent used for the production of the  $KUF_5$  may be formic acid, sucrose, oxalic acid or other suitable, preferably organic, reducing agent. The equation when using formic acid is as follows:



40 When using sucrose or cane sugar, that material is first hydrolyzed in acid to produce glucose and fructose in accordance with the following equation:



The glucose and fructose then act as reducing agents in the production of potassium uranous fluoride.

When oxalic acid is used as a reducing agent, 50 potassium uranous fluoride is produced in accordance with the following equation:



55 It will, of course be understood that the above

equations are merely illustrative of reducing actions for the production of potassium uranous fluoride.

Sucrose is preferred as the reducing agent, as the rate of precipitation of potassium uranous fluoride is increased by more than 15% over that obtained with formic acid. However, there is more discoloration when using sucrose, which discoloration is of course undesirable, as excluding some of the light needed for reduction.

In more detail, our process is carried out in the trays 11, 12, 13, 14, 15, 16 and 17.

The trays illustrated in the drawing are intended to be 10 x 12 feet in plan and filled to a depth of 4". This would make approximately 1080 liters per tray. The reagents required per tray are as follows:

|                                                                 | Original<br>Filling<br>Metric<br>Units | English<br>equiv. | Refilling<br>Metric<br>Units | English<br>equiv. |
|-----------------------------------------------------------------|----------------------------------------|-------------------|------------------------------|-------------------|
| 1. Total Volume.....                                            | 1,080 l.....                           | 285 gal.....      |                              |                   |
| 2. $\text{UO}_2(\text{NO}_3)_2 \cdot 6\text{H}_2\text{O}$ ..... | 108 kg.....                            | 237 lb.....       | 108 kg.....                  | 237 lb.           |
| 3. $\text{KF} \cdot 2\text{H}_2\text{O}$ .....                  | 43.2 kg.....                           | 95 lb.....        | 61.2 kg.....                 | 135 lb.           |
| 4. HF 30%.....                                                  | 144 l.....                             | 362 lb.....       | 28.8 l.....                  | 72 lb.            |
| 5. $\text{HCOOH}$ (formic acid).....                            | 30.24 l.....                           | 8 gal.....        | 8.34 l.....                  | 8.75 gts. or      |
| 6. $\text{C}_{12}\text{H}_{22}\text{O}_{11}$ (sucrose).....     | 74 kg.....                             | 163 lb.....       | 74 kg.....                   | 163 lb.           |

The amount of potassium uranous fluoride, which will be called for convenience "green salt," which is produced per day is dependent upon the amount of sunlight.

Two days of sunlight in the spring and summer months at New Jersey latitudes are required for conversion of 90% of the nitrate to potassium uranous fluoride. A good sunny day, using the equipment disclosed, should produce about 150 grams of "green salt" per sq. ft. of tray area. This makes it possible to produce from 200 to 400 lbs. of green salt per day, depending on the ultra-violet intensity of the sunlight. It has been determined that all of the ultra-violet component of the sunlight is utilized in the precipitation of the "green salt" as well as visible components including up to approximately 4300 Angstrom units.

The actual quantities and ratios of the various reagents used for the production of  $\text{KUF}_5$  may vary, depending upon the desired method of handling, and weather conditions. For example, in cold weather, it may be desirable to reduce the charge shown in the above table by as much as 50% in order to reduce the amount of the yellow scale formed.

While other halides of tetravalent uranium such as  $\text{UF}_4$  or  $\text{UCl}_4$  may be used in the electrolysis process described below, unless they are very pure the preparation of  $\text{KUF}_5$  in the manner described has certain advantages when uranium metal of high purity is desired. The precipitation of  $\text{KUF}_5$  in the manner described results in the removal of certain impurities which are present in the normal commercial grade of uranyl nitrate, resulting in a potassium uranous fluoride of high purity which in turn may be electrolyzed as hereinafter described to a very pure metal. The process is thus of great value when halides of tetravalent uranium of the desired chemical purity are not available commercially.

Other uranous fluorides such as  $\text{NaUF}_5$  may be produced by a process similar to that described by changing the proper reagents, as substituting sodium fluoride for potassium fluoride.

The trays are first partially filled with water (or with supernatant liquor from a previous simi-

lar operation) and the desired quantities of potassium fluoride, hydrofluoric acid, and a reducing agent such as sucrose dissolved therein. Uranium nitrate is dissolved in its own weight of water and the concentrated solution added to the liquor in the trays. It is undesirable to add the concentrated reagents to the nitrate solution or to dissolve the solid nitrate in the solution of the other materials.

On cool days a yellow precipitate or scale is obtained, which is, however, soluble in hot water, with conversion to nitrate solution and  $\text{KUF}_5$ . It is necessary, therefore, in case this salt separates, to dissolve it by agitating it in hot water and then filtering and proceeding as directed for potassium uranous fluoride.

When the reaction has reached the desired

degree of completion, the supernatant liquid is 30 decanted into the next lower tray and the precipitated potassium uranous fluoride washed from the trays. The suspension is passed through a filter 18 and washed with distilled water and alcohol. In order to increase the rate 35 of filtration a vacuum connection 21 is desirably made to the container 22 which holds the filter 18. The salt is then dried in air, as in an oven 23, at about 110° C. Water 19 from filtration of green salt is discarded.

In accordance with the drawing it will be seen 40 that we propose to start with full charges of the green-salt-producing bath in trays 11 to 14, inclusive, while allowing the uranium content to gradually deplete in trays 15, 16 and 17 by failure to add any more uranium nitrate to these 45 trays. After recharging the sugar-containing solutions four times, it is considered necessary to discard the entire batch due to discoloration of the oxidized reducing agent.

The solution, depleted by precipitation of 50 potassium uranous fluoride, contains some potassium nitrate and considerable hydrofluoric acid and potassium fluoride. To the trays containing uranium depleted solutions, that is, those numbered 12 to 14, inclusive, which are to 55 be maintained up to strength and which successively receive the solutions from the preceding ones of lower numbers, one mol of formic acid, or  $\frac{1}{6}$  mol of sucrose, together with 3 mols of potassium fluoride, and 2 mols of hydrofluoric acid 60 are added for each mol of uranyl nitrate. This formula has proven satisfactory but we do not wish to be limited to these proportions.

As an alternative, di-potassium uranous fluoride,  $\text{K}_2\text{UF}_6$ , produced by a process described in 65 the copending application, Serial No. 478,271 filed March 6, 1943, by John W. Marden and Rudolf Nagy, may be used in place of potassium uranous fluoride. The metal produced from this salt is in every way comparable with that produced from  $\text{KUF}_5$  and  $\text{UF}_4$ .

#### Electrolysis of "green salt"

The electrolysis of "green salt" to produce 75 uranium powder may be carried out in furnace

24 consisting of a graphite crucible 25 and a molybdenum electrode 26. The crucible and electrode are connected to a source of direct current 27 so that the crucible is the anode and the electrode 26 the cathode. Means may be provided for heating the contained electrolyte, other than by the electrolysis current between the electrodes, such as resistance windings about the crucible (not shown). However, we have found that the desired results may be obtained by heating the electrolyte with the electrolysis current only.

The electrolysis process consists of fusing a mixture of sodium and calcium chlorides in a crucible 25, adding to said fused mixture the desired proportion of "green salt," and electrolyzing the bath until the uranium is deposited on the cathode. Using a battery of five furnaces with crucibles 9" inside diameter and 21" deep, with an effective volume of approximately 1300 cu. in. on three eight-hour shifts, approximately 250 lbs. of metal powder per day may be produced. For each furnace, 1800 amperes of current with electrode changes every 60 minutes are required.

The crucibles are charged with metal halide salts desirably initially charged with a mixture consisting of about 80% calcium chloride by weight and about 20% sodium chloride. A total of 80 to 100 pounds is required.

If the salts are not fused by external heating, an auxiliary or "dummy" electrode may be used. The use of a dummy electrode during charging serves not only for the heating but also for the removal of deleterious impurities in the bath such as iron and boron prior to electrolysis. Such impurities are deposited on the dummy during the charging operation or volatilized from the bath by the heating.

The bath is heated to the temperature of approximately 950° C. by the passage of current and the crucible filled to within 6" of the top. When all the salt is melted about one pound of "green salt" is added to the crucible. About five minutes after the addition of green salt the original electrode, now called the "dummy," is removed.

About seven pounds of "green salt" are then added to the bath and the melt allowed to stand until the temperature of the bath falls to 900° C. A clean electrode is then introduced into the bath and the electrolysis carried to completion. Allowing the melt to stand without electrolysis serves to eliminate any volatile deleterious materials, such as boron which passes off as a halide or mixture of halides, from the bath prior to electrolysis.

The amount of uranium salts initially added to the fused chlorides should be of the order of 1/2% to 3% of the total weight of the chlorides in the crucible. The amount of uranium salts added after the dummy cathode is removed from the crucible should be of the order of 5% to 15% of the total weight of the chlorides in the crucible.

One batch of metal powder made from several first electrodes contained more than 15 parts per million of boron. Powder made from corresponding second electrodes averaged about 1/2 part per million. Powder made by similar operations, except that one electrode was used for both the charging and the electrolysis averaged 1 to 3 parts per million of boron. For certain purposes a minimum boron content is desirable.

If external heat has initially been applied to fuse the bath, the intensity thereof must be

reduced while the cell is in operation because of the energy dissipated by the electrolysis current, as the temperature must be held at 900° C. ±25° C. throughout a run. Low temperatures result in large deposits of salts on the electrodes but low yields because of the fineness of deposited powder.

The idea disclosed in Fig. 1 is to introduce the "green salt" into the fused bath by throwing it on top of the surfaces of said bath. If the salt is potassium uranous fluoride or uranous fluoride, it may oxidize to some extent before becoming completely dissolved. Once dissolved it is protected by the fused bath and no oxidation seems to take place. When the salt can be plunged directly below the surface it is heavier than the calcium chloride or sodium chloride bath and sinks to the bottom where it is dissolved without oxidation.

20 In accordance with Fig. 2 we propose to introduce the dry salt below the surface of the bath by weighing the desired amount into a tube 44 with a hinged cover 45 at its lower end and initially closed, as shown in full lines. A plunger 25 46 is inserted into the tube with the "green salt" or other compound to be electrolyzed, placed in the bath 28<sup>a</sup> in the crucible 25<sup>a</sup>, and said salt expelled beneath the surface after dropping the cover 45, as by operating the rod 47 connected to a crank 48 thereon. We have simplified the showing by omitting the electrode.

25 Fig. 3 shows alternative apparatus for introducing "green salt" in the form of a pressed mass 49 beneath the surface of the electrolyte bath 28<sup>b</sup> in crucible 25<sup>b</sup>, as by holding it in tongs 51 and forcing it quickly below the surface.

30 In Fig. 4 we have shown further alternative apparatus, for introducing "green salt" by means of a small screw type conveyor 52 operating in a cylindrical extension 53 on the bottom of a hopper 54 containing the desired quantity of salt which is introduced into the bath 28<sup>c</sup> from the lower open end 55 of said extension 53. The screw conveyor member 52 may be operated through suitable gearing by means of an electric motor or other power means 56. In all forms of our invention illustrated in Figs. 2, 3 and 4 the parts of the apparatus which come in contact with the fused bath are desirably made of molybdenum or some such material in order to avoid contaminating said bath.

35 Still another means of introducing "green salt" without oxidation is to place a cover 57 of asbestos, or other halide-resistive insulating material, over the crucible 25<sup>d</sup> and flow inert or protective gas such as argon or hydrogen, onto the surface of the bath as by means of a valve-controlled pipe 58, to prevent oxidation of the uranium salts or metal during the process of introducing the salt from the bottom of hopper 59. Holes 61 may be provided in the cover 57 to allow for the escape of gas generated during the electrolysis operation and as vents for the protective gas. A valve-controlled branch 62 of the pipe 58 might serve as a means for introducing gas to control or expedite the flow of the salt from the hopper 59. Another valve-controlled branch 63 might be employed to keep a protective atmosphere over the top of the salt, a cover 64 with a valve-controlled vent pipe 65 being in such instance provided for the hopper 59.

40 The cathode 26 is lowered into the bath to within 2" of the crucible bottom and the electrolysis current of about 1800 amperes started and maintained for about 60 minutes.

The furnaces or crucibles previously described for fused salt electrolysis, in accordance with our invention, are of the single unit type, that is, the same crucible is set in insulation and a single electrode placed in the center thereof. Any number of these furnaces may be operated together in series or in parallel, but each is an individual unit. When an electrode is changed in a single unit type, the furnace must be shut off or shunted out. In very large installations such construction is not suitable because the electrode becomes very large and the cathode to crucible spacing is too great. Handling the electrode then becomes a problem and the voltage required to operate the furnace is increased.

For operations on a large scale where the metallic deposit is removed on the cathode, a furnace with several cells built together, as illustrated in plan in Fig. 6, is desirable. The crucible 25<sup>e</sup>, which also serves as the anode, in this instance is elongated and provided with baffles or partitions 66, said baffles projecting alternately from the opposite long sides 73 and 76 of the crucible. As in the previous instance, a suitable conductive material, such as carbon or graphite, must be used. An electrode 26<sup>f</sup> to function as a cathode is suspended in each compartment, except the first or melting compartment 67, and all connected together, as illustrated, so that the entire unit behaves as several cells connected in parallel.

The operation of such apparatus may be to charge a substantial quantity of the salts to make up the fused bath each time the uranium salts to be electrolyzed are added. These salts may be charged into the end compartment 67, where they are melted, as by alternating current between dummy electrodes 68 and 69. The molten salt will then flow into section 71, through space 72 between partition 66 and the long wall 73 of the assembly toward which it projects. From section 71 it would flow on to section 74, through space 75 between the next partition 66 and the long wall 76 toward which it projects. From thence it would flow on to the remaining sections or compartments in a similar manner.

Uranium salt to be electrolyzed is added to each section except the first and last, from time to time. In the last section no uranium salt is added, this being used to take out the last trace of uranium before the salts run to the overflow pipe 77. The electrodes may be removed one at a time whenever sufficient deposit has been collected. Momentary interruption of the current in one section does not materially effect the operation of the battery as a whole, as the other electrodes would carry the extra current for a short while. Such a furnace is particularly useful for operations where a large amount of make-up bath salts must be used. It avoids loss of uranium in the discharge and makes the process substantially continuous. Current limiting devices may be incorporated for use with the arrangement. Especially where it is not necessary to recharge the bath, the first section designated 67 may also be used for electrolysis like one of the single unit type furnaces previously described.

Referring now to the embodiment of our invention illustrated in Fig. 7, there is shown a crucible 25<sup>f</sup>, which may be like a single unit crucible 25 or a multiple unit crucible 25<sup>e</sup>, containing a fused salt electrolyte bath 28<sup>f</sup> and in which is suspended a special type of electrode 26<sup>f</sup> to function as a cathode. The reason for

the special type illustrated is that while molybdenum is at present the most suitable metal for the cathode, it is heavy and difficult to fabricate. For best results such a cathode should have a large diameter and surface area, without excessive cross sectional mass. A hollow cylinder satisfies these conditions, but the fabrication of such a cylinder of sufficiently large dimensions out of molybdenum is difficult.

It is, therefore, desirable to construct a cathode with a surface of molybdenum on a base metal which may be readily shaped as desired. Thin cylinders of molybdenum, such as might be constructed of sheet metal, do not have sufficient mass to conduct the heavy currents used in electrolysis furnaces. In accordance with our invention we, therefore, propose to make the electrode 26<sup>f</sup> as a hollow cylinder 78 of steel or other suitable metal, closed at its lower end as indicated at 79, and coated or sheathed from the bottom to above the top surface of the electrolyte bath with molybdenum 81. The molybdenum is desirably applied as a continuous sheet or cup over the core 78, or as a ribbon or wire wound helically on the tube 78, so that the adjacent edges thereof abut and are thereafter desirably welded together so as to form, in effect, a continuous molybdenum surface. Such an electrode has the advantage of a large molybdenum surface, light weight, and a sufficient but not excessive cross sectional area. Covered electrodes of the type mentioned above are disclosed and claimed in the copending application of William C. Lilliendahl and Donald Wroughton, Serial No. 517,016, filed January 5, 1944, now abandoned.

The assembled electrode 26<sup>f</sup> may be supported in a head forming a flange 82 from which a pipe 83 extends and connects with a port 84 to the interior of the cylinder 78. The upper end of the cylinder is closed by a cap 85 carrying a pipe 86 of steel or other suitable material, which extends down to near the bottom of the cylinder 78, and through which air or other fluid may be introduced to said cylinder for cooling the electrode when desired, as during withdrawal from the bath, in order to minimize oxidation of the deposit. The cooling fluid would pass down the pipe 86 and return between the pipe and the cylinder 78 through the port 84 and out of the pipe 83, thereby effecting the desired cooling action.

When using a cathode in the form of thin strips, a cylinder, or rectangular rod of molybdenum, it is found that when operated in a crucible of the design shown in Figs. 1 to 7, inclusive, the deposit is non-uniform. That is, the rate of deposition at the top portion of the electrode, or near the surface of the bath, is faster than at the lower portion. This results in a cone-shaped deposit, as shown in Fig. 1, on the electrode 25. This condition of unequal distribution is most pronounced in electrodes of small cross sectional area.

Such a deposition is objectionable because it has a tendency to peel due to the weight of the deposit formed and sometimes results in loss of deposit. The formation of such deposits also reduces the electrolyzed metal weight per unit area of cathode surface, which in turn limits the charge per run of material electrolyzed, thus reducing the yield per man hour of operation. The condition appears to be due to the relatively large voltage drop in the electrode. In operation, this

may be of an order of magnitude of one to two volts.

As electrolysis starts, the voltage drop across the bath to the lower portion of the cathode is less than at the top, which results in increased deposit at the top of the electrode. This may also be due to convection currents of the electrolyte. As electrolysis proceeds, the deposit builds up at the top of the bath so that the resistance at that point decreases, resulting in further increase in the rate of deposition at the top of the electrode at the expense of the lower portion.

This condition of unequal deposition may be prevented by tapering or forming the crucible 25<sup>a</sup> with an inverted frusto-conical interior, so that the current along the cathode 26<sup>a</sup> is uniform throughout the submerged length, as shown in Fig. 8, or by having the cathode 26<sup>b</sup> flare downwardly, or with its lower portion frusto-conical, in a crucible 25<sup>b</sup> of uniform cross section throughout its height, as shown in Figs. 9 and 10, or by tapering the crucible to some extent and flaring the cathode to some extent, whereby the distance between the cathode surface and the crucible surface steadily decreases from the top of the bath to the bottom of the cathode, the rate of decrease being sufficient to balance the drop along the cathode, in order to equalize the current between cathode and crucible and result in uniform thickness of deposit, as illustrated in Figs. 8, 9 and 10.

The cathode 26<sup>b</sup>, illustrated in Figs. 9 and 10, may be formed of two molybdenum plates, trapezoidal in shape, with their widened portions bulged or formed as hollow flanged half-cones 87 and 88, and then connected together as by molybdenum bolts 89. Current leads 91 are provided for introducing the electrolysis current to the electrode. When the electrolysis operation is completed the electrode may be withdrawn from the bath as usual, and after cooling the plates separated by removing the bolts, thereby facilitating the removal of the deposit from both inside and outside. The upper bolts 89 (Fig. 9) are not immersed in the bath and are easily removed. However the lower bolts acquire a coating during electrolysis that must be removed before disassembly of the electrode plates. The shape illustrated is not only conducive to a uniform deposit, but is more effective for preventing any slippage of the deposit by virtue of the vertical component of the pressure between the deposit and the cathode, acting to support said deposit. Tapered electrodes of the type mentioned above are disclosed and claimed in the copending application of Towson Price, Serial No. 510,557, filed November 16, 1943, now abandoned.

Operation of the electrolyte bath at about 900° C. is an improvement over prior electrolysis processes in which operation was effected at lower temperatures, in that the proportion of metal fines is decreased and a coarser uranium powder produced, which is less pyrophoric.

If a hollow electrode, as disclosed in connection with Fig. 7, is employed, it is also desirable in accomplishing the above results to inject a rapid stream of air through it during the operation of raising said electrode from the bath, thus assisting in the solidification of salts on the cathode to form a protective layer on the removed metal.

As a result of the improved process involving an increase in the electrolyte temperature of

approximately 100° C., it has been found that said metal does not have the pyrophoric properties which are present in powders when baths are operated at 800° C.

5 The melting point of uranium is relatively low, that is approximately 1150° C. With baths operating at 875° C. to 950° C., the actual temperature at the cathode is materially affected by current density and cathode potential, which is in turn affected by bath composition. It has been discovered that, by a proper control of the variables, uranium metal is produced on the cathode in such a compact form that the deposit can be removed, washed with water, and the coherent 10 metalized, sintered, mass fused in vacuo, thereby eliminating the necessity of the washing and grinding operations later fully disclosed.

The electrochemical equivalent of tetravalent uranium is 2.22 grams per ampere hour. The 7 20 pounds of "green salt" contain 2020 grams of uranium, which would require 910 ampere hours at 100% efficiency. In practice, however, approximately 1800 ampere hours are required for 7 pounds of "green salt." The current efficiency 25 does not appear to be appreciably affected by current density at the cathode. The most convenient combination of current and time which will yield 1800 ampere hours for that size charge can be used, but the current strength must be 30 that required for keeping the furnace at the desired temperature.

At the completion of the run, the cathode is desirably taken quickly from the bath for removal of the deposit. It is then preferably immediately placed in a tall cylindrical vessel 92 with a funnel shaped top 93, as shown in Fig. 11, which is then at once filled with dry salt, such as dry sodium chloride, anhydrous calcium chloride, or similar material 94. The salt is partly 35 melted on the surface of the electrode, sealing the metal particles and preventing oxidation. If a hollow air-cooled electrode 26<sup>f</sup>, as shown in Fig. 7, is used, then it may not be necessary to use the enclosing receptacles 95 containing cooling 40 means, such as water 96, which is introduced by pipe 97 and overflows from pipe 98.

However, for the ordinary type of electrode 26<sup>j</sup> shown in Fig. 11, the external cooling means is desirable as it facilitates the operation by effecting a quicker cooling. The purpose of this treatment is to prevent oxidation while the deposit cools. Other methods of accomplishing the result, such as quickly redipping in the bath after partial cooling, or pouring some of the electrolyte over the withdrawn cathode after partial cooling, have also been used successfully. Use of this improved technique of salt smothering has enabled us to substantially increase the average yield.

60 At the end of an electrolysis run, enough salt should be removed from the bath so that 12 to 15 pounds (that is about 15% of the total charge of fresh salt mix), of 90% calcium chloride and 10% sodium chloride, may be added to the crucible. Some salt is always removed on the electrode and the rest may be dipped from the molten bath, as by means of a suitable cup. The furnace is then charged, preferably using the dummy electrode as described, and the operation 65 repeated.

We do not wish our invention to be limited by the specific dimensions of the furnaces as given above. Other sizes of furnaces have been used for carrying out the same process with good results. Also bath temperatures between 750° C.

and 950° C. will yield uranium metal, although 900° C. is the preferred temperature since, other factors being equal, operation at 900° C. has been shown to result in an increase in yield of usable metal powder.

The bath composition may vary considerably from the original charge, i. e. 80% CaCl<sub>2</sub>-20% NaCl, with good results. The bath described is desirable because it has a sufficiently low melting point and requires a minimum amount of recharging to preserve fluidity.

Furthermore, halides of tetravalent uranium other than KUF<sub>6</sub>, such as UF<sub>4</sub> and UCl<sub>4</sub>, may be electrolyzed in the same bath. Uranium tetrafluoride, (UF<sub>4</sub>) for example, has the advantage that it gives a better material yield than KUF<sub>6</sub>, based upon the uranium content. Whenever it can be obtained in the required degree of purity it then becomes the preferred uranium salt. When using UF<sub>4</sub>, it is desirable to recharge the furnaces with an 80% CaCl<sub>2</sub>-20% NaCl mixture rather than with the 90% CaCl<sub>2</sub>-10% NaCl mixture used with KUF<sub>6</sub>. This compensates for the potassium content of the KUF<sub>6</sub>.

In all cases where the fluoride salts of uranium are used for electrolysis, it is necessary to discard a certain fraction of the bath at frequent intervals to remove part of the fluorides from the bath. For best results, the calcium fluoride content should not exceed 30%, although good yields of metal have been obtained from baths containing as much as 40% CaF<sub>2</sub>. A bath which gave very good results, for example, was composed of 18.7% CaF<sub>2</sub>, 60.8% CaCl<sub>2</sub>, and 10.5% NaCl+10% KCl after all the uranium salts had been electrolyzed.

However, when operating the electrolyte bath at about 900° C., the electrolyte is very fluid even with high percentages of calcium fluoride. We have, therefore, been able to use the same bath continuously for more than 15 times with no removal of electrolyte, as by dipping. Salts, generally calcium chloride and sodium chloride, as in the ratio of 4 to 1, are added but only to compensate for what is lost by evaporation and removal on the electrode.

Baths operated continuously, as described, are considered superior to periodically replaced baths in the following respects:

- (1) Contamination by iron is minimized.
- (2) The amount of calcium chloride and sodium chloride used in the process is substantially reduced.
- (3) The dangers attending dipping are eliminated.
- (4) The power necessary for heating the recharged bath is saved.
- (5) The oxides produced in the bath, due to heating by electrolysis current are eliminated. Such oxides increase the melting point, and induce slipping and poor yields of metal.
- (6) More runs per day can be made.
- (7) Larger charges of uranium salts can be used, thus increasing the electrical efficiency.
- (8) More than one electrode can be used in a bath with alternate removals.

As an alternative, to the use of the dummy electrode, the salt charge may be melted in an auxiliary furnace and poured into the electrolysis cell when molten. In such cases, a dummy electrode need not be used if the salts are of satisfactory chemical purity.

pure metal powder by a process which consists essentially of crushing and grinding said deposits, and washing and rinsing the crushed and ground material until the residue is of the desired fineness and substantially free of deleterious substances, such as salts from the electrolysis bath and finely divided uranium metal and oxide.

The electrode deposit as removed from the bath consists of metal powder and solidified salts which serve to protect the metal from oxidation. The ratio of salt to metal powder depends on the temperature and composition of the bath, high temperature and low viscosity favoring a low ratio of salt to metal powder. Operating at 875° C. to 900° C., the ratio of salt to metal is approximately 2 to 1.

The handling of the cathode and its deposit after removal from the bath may, for example, be divided into several unit operations, which

comprise:

1. Removal of deposit from the cathode, as by means of an air hammer 29 or a cold chisel.
2. Coarse crushing to 4 mesh or finer, as by means of a jaw crusher 31.
3. Fine crushing, as by means of a roller crusher 32.
4. Water washing to remove soluble salts, as in a tumbling barrel 33.
5. Wet grinding to break up aggregates and assist in the removal of insoluble salts, as by means of disk grinder 34.
6. Further washing, which may include the use of acetic acid, to remove salts retained from previous operations, as in a tumbling barrel 35, followed by repeated decantation.
7. Filtration of metal powder followed by washing with 90% alcohol and ethyl ether, as in vacuum filters 36.
8. Drying in vacuo and preserving in an atmosphere of inert gas, as in vacuum ovens 37.

For producing uranium of extreme purity, all operations should be conducted in equipment composed of non-contaminating material, such as wood or hard rubber, where practical, and the grinding and crushing equipment made of steel, to reduce the pick-up of foreign elements. Hard glass which might contain borates is to be particularly avoided and where the use of glass equipment is necessary, silica or lime glass should be used. The steps previously noted will now be discussed in detail with respect to the practice for large scale production.

For handling deposits comprising 250-300 lbs. of metal powder per day, a jaw crusher capable of handling 900 lbs. of material per day is required. The crusher should have an effective jaw opening of approximately 1/4".

After passing through the coarse jaw crusher 31 the material is passed through the roller crusher 32 set at approximately 0.100" and then transferred to a wooden tumbling barrel 33, rotating at from 60 to 80 R. P. M., and provided with suitable mechanism for tipping to obtain rapid washing by decantation. Sufficient distilled water is added to dissolve the soluble salts and the barrel rotated for a period of 20 minutes. Considerable heat is evolved during this operation, due to the solution of the calcium chloride contained in the deposit, and it is necessary to cool, as by the addition of ice. The temperature of the solution should be maintained below 30° C. during this operation to avoid oxidation of the uranium powder. Approximately 8 liters of distilled water are required per pound of metal pow-

#### Conversion of electrode deposit

The deposit on the electrode is converted to

der in the deposit, to which 2 to 3 lbs. of ice are added.

After completion of the tumbling, the barrel is tipped and the metal sludge washed three times by decantation, rotating two to three minutes between each operation. The wash liquors should be recovered and settled, as the uranium metal fines and oxides should be reconverted to nitrate for subsequent precipitation as "green salt" in order to avoid loss of valuable material.

The metal sludge after removal from the tumbling barrel is run wet through a disk grinder 34 to break up aggregates and assist in further removal of insoluble oxides and fluorides. A grinder capable of yielding material between 50 and 100 mesh is required for satisfactory removal of the insoluble materials. Particles coarser than 50 mesh interfere with successful removal of impurities in the washing to follow.

The ground material is transferred to the rotating barrel 35 and washed with water. After rotating for 10 minutes, the barrel is tilted and the light impurities poured off. This process, tumbling for 2 to 3 minutes and pouring off, is repeated with distilled water until the supernatant liquid is free from light material, such as  $\text{CaF}_2$ . In some cases a 2% solution of acetic acid may be used, in one of the early washes to assist in the process.

The metal powder is then transferred to a suction filter of the Buchner type and the filtration facilitated by a connection to vacuum line 39. The metal on the filter is desirably washed twice with 95% ethyl alcohol, using sufficient reagent to cover the sludge and draining between additions. The powder is then desirably washed twice with ethyl ether, acetone or other volatile solvent, and after partial drying is immediately transferred to tared cans and placed in vacuum ovens 37. After drying in vacuum for eight hours, the ovens are filled with an inert gas such as nitrogen, carbon dioxide or argon, but preferably with the latter, and the metal powder preserved therein until ready for the pressing operation. However, the long vacuum oven drying may be omitted, if desired, as the powder can be sufficiently dried on a suction filter after washing with a volatile solvent. To reduce fire hazard, the metal powder should never be handled in lots larger than about 10 lbs., especially after washing with ether or acetone.

Further operations may involve consolidating the metal powder in press 41 and finally sintering and fusing, or otherwise heat treating, in furnaces 42, as in accordance with Patent No. 1,814,719.

From the foregoing it will be seen that we have devised an improved method comprising first purifying the raw material by transforming to an oxygen-free fluoride, while simultaneously avoiding contamination with deleterious materials, particularly boron, and after electrolysis preventing subsequent contamination and oxidation, using only water which is distilled, so that the uranium metal powder when finished is suitable for subsequent processing to form pure metal articles of the desired shapes.

Although preferred embodiments of our ideas have been disclosed, it will be understood that modifications may be made within the broad spirit and scope of the invention.

We claim:

1. The method of producing pure uranium powder that comprises introducing a single uranous halide selected from the class consist-

ing of potassium uranous fluoride, uranous fluoride and uranous chloride into a carbon crucible containing a fused bath consisting of approximately 80% calcium chloride and 20% sodium chloride by weight and having a molybdenum element therein, the uranous halide being introduced in an amount approximating 5% to 15% by weight of the fused bath, electrolyzing at a temperature of approximately 900° C. with the crucible as anode and the molybdenum element as cathode to deposit uranium on said cathode, removing the coated cathode, permitting the cathode to cool, removing the deposit therefrom, and crushing, washing and drying said deposit to produce pure uranium powder.

2. The method of producing pure uranium powder that comprises introducing potassium uranous fluoride into a carbon crucible containing a fused bath consisting of approximately 80% calcium chloride, and 20% sodium chloride by weight and having a molybdenum element therein, the potassium uranous fluoride being introduced in an amount approximating 5% to 15% by weight of the fused bath, electrolyzing at a temperature of approximately 900° C., with the crucible as anode and the molybdenum element as cathode to deposit uranium on said cathode, removing the coated cathode, permitting the cathode to cool, removing the deposit therefrom, and crushing, washing and drying said deposit to produce pure uranium powder.

3. The method of producing pure uranium powder by electrolysis in a continuously operating bath that comprises introducing potassium uranous fluoride into a carbon crucible containing a fused bath consisting of approximately 80% calcium chloride and 20% sodium chloride by weight and having a molybdenum element therein, the potassium uranous fluoride being introduced in an amount approximately 5% to 15% by weight of the fused bath, electrolyzing at a temperature of approximately 900° C. with the crucible as anode and the molybdenum element as cathode to deposit uranium on said cathode, removing the coated cathode from the crucible, removing a portion of said bath and refilling said bath to its original level with a mixture consisting of approximately 90% calcium chloride and 10% sodium chloride, the portion removed being such that the addition of the mixture in an amount approximating 15% by weight of the original fused bath will restore the bath to its original level, introducing a new charge of potassium uranous fluoride into the refilled bath and electrolyzing at a temperature of approximately 900° C.

#### References Cited in the file of this patent

#### UNITED STATES PATENTS

| Number    | Name            | Date          |
|-----------|-----------------|---------------|
| 596,458   | Inglis          | Dec. 28, 1897 |
| 618,575   | Lyte            | Jan. 31, 1899 |
| 808,066   | Borchers et al. | Dec. 26, 1905 |
| 850,376   | Kugelgen et al. | Apr. 16, 1907 |
| 1,077,894 | Stevens         | Nov. 4, 1913  |
| 1,197,137 | McNitt          | Sept. 5, 1916 |
| 1,255,197 | Malm            | Feb. 5, 1918  |
| 1,534,319 | Hoopes et al.   | Apr. 21, 1925 |
| 1,646,734 | Marden          | Oct. 25, 1927 |
| 1,814,719 | Marden et al.   | July 14, 1931 |
| 1,821,176 | Driggs et al.   | Sept. 1, 1931 |
| 1,826,806 | Marden et al.   | Oct. 13, 1931 |

(Other references on following page)

## UNITED STATES PATENTS

| Number    | Name          | Date          |    |
|-----------|---------------|---------------|----|
| 1,835,026 | Driggs        | Dec. 8, 1931  |    |
| 1,842,254 | Driggs        | Jan. 19, 1932 | 5  |
| 1,861,625 | Driggs et al. | June 7, 1932  |    |
| 1,874,090 | Driggs        | Aug. 30, 1932 |    |
| 2,045,073 | Eldridge      | June 23, 1936 |    |
| 2,059,468 | Lyons         | Nov. 3, 1936  |    |
| 2,068,005 | Dandt et al.  | Jan. 19, 1937 | 10 |

## FOREIGN PATENTS

| Number  | Country | Date          |  |
|---------|---------|---------------|--|
| 366,523 | France  | July 30, 1906 |  |

## OTHER REFERENCES

Driggs et al., article in Industrial and Engineering Chemistry, May 1930, pp. 516-519.

Smyth, "Atomic Energy for Military Purposes," page 27, para. 2.27, August (1945).

Goodwin, "Electrolytic Calcium" in Proceedings of the American Philosophical Society, vol. 43, pages 383 and 384 (1904).

Croghins, Unit Processes in Organic Synthesis, published 1938 by McGraw-Hill Book Co. Inc., page 604.

Morrow, Biochemical Laboratory Methods, published 1927 by John Wiley and Sons Inc., page 191.